

C. E. ARNOLD.

PROCESS OF PRODUCING ARTIFICIAL LEATHER.

APPLICATION FILED SEPT. 3, 1914.

1,277,528.

Patented Sept. 3, 1918.



Witnesses:

A. D. McLaughlin  
J. Kosler.

Inventor

Charles Elwood Arnold

By his Attorneys  
Pringle, Wright & Snell

# UNITED STATES PATENT OFFICE.

CHARLES ELWOOD ARNOLD, OF WILMINGTON, DELAWARE, ASSIGNOR, BY MESNE ASSIGNMENTS, TO E. I. DU PONT DE NEMOURS AND COMPANY, A CORPORATION OF DELAWARE.

## PROCESS OF PRODUCING ARTIFICIAL LEATHER.

1,277,528.

Specification of Letters Patent.

Patented Sept. 3, 1918.

Application filed September 3, 1914. Serial No. 859,964.

*To all whom it may concern:*

Be it known that I, CHARLES ELWOOD, ARNOLD, of Wilmington, in the county of New Castle, and in the State of Delaware, have 5 invented a certain new and useful Improvement in Processes of Producing Artificial Leather, and do hereby declare that the following is a full, clear, and exact description thereof.

10 My invention relates particularly to an improvement in the method of producing coated fabrics but more especially woven fabrics carrying a coating or layer of a nitro-cellulose composition.

15 The object of my invention is to produce a product of this kind in which the layer of composition carried by the fabric will be very effectively and securely anchored on the fabric and in which the coating composition 20 will adhere in an effective manner to the fabric.

25 More specifically the object of my invention is to produce goods of the quality stated without the use of a special cementing coat and to provide the total thickness of coating in one operation.

30 While my invention is capable of embodiment in many different forms, for the purpose of illustration, I shall describe only one form thereof and have shown one form of apparatus with which my invention may be carried out, in the accompanying drawings, in which—

35 The figure is a diagrammatic side elevation showing an apparatus that may be used in carrying out my invention.

Referring to the drawing I have provided a shaft 1 carrying a shell 1<sup>a</sup> on which the roll of goods is carried. The shaft is provided 40 with any suitable device to insure that the goods being pulled off the roll will be taut. The goods pass from the shell 1<sup>a</sup> over two supporting rolls 2 and 5. Between these supporting rolls there is a doctor or smear-on 45 blade 4 in front of which is carried a body of plastic or paste 3 containing a solvent. The goods thus treated pass into an evaporating chamber 6 in which the major portion of the solvent is evaporated and re-50 covered. It is undersirable to evaporate the entire amount of solvent as the coated goods when leaving the same pass to calendering rolls 7, where it must be in a pliable condition. The object of the calendering rolls 7

is to give the coated fabric a uniform thickness and render the coating smooth. They need not be very large or heavy rolls as the plastic after coming from the drying chamber is properly coated and anchored to the fabric but on account of the method of applying the coating in the form of a paste the goods are somewhat too rough to emboss, and the rolls 7 are used simply to smooth the plastic and give the desired uniformity of thickness. The rolls 7 may also be engraved 65 so as to give an embossed pattern on the goods, thereby serving the double purpose of gaging and embossing the goods. I have also provided a winder 8 which may be so constructed as to wind up the finished product 70 and keep the tension on the goods through the entire train of the apparatus.

In preparing coated fabrics by the well known coating machine, which consists of a doctor blade and a drying device, it is 75 customary to obtain the desired thickness of coating by applying a number of successive layers or coatings and evaporating the solvent after each application. If a coating of the total thickness desired is applied at 80 one time in order to reduce the number of operations the product is not satisfactory because of pin-holes that are formed when the solvent is evaporated. I avoid this difficulty by using a thicker, that is, pasty 85 coating material and preferably pass the coated material between calendar rolls before all the solvent has been evaporated. The composition may be any suitable nitro-cellulose composition containing volatile 90 solvents. It may also contain any suitable oil or pigment. This calendering operation reduces the coating to a uniform thickness and eliminates the pin-holes. Furthermore 95 by my process the coating is firmly anchored to the fabric because the coating material when applied contains sufficient solvent to enable it to penetrate the interstices of the fabric.

While I have described my invention in 100 detail I wish it to be understood that many changes may be made therein, without departing from the spirit of my invention.

I claim:

1. The process of producing a coated fabric which comprises applying to a fabric a coating of a film-producing composition in the form of paste containing a solvent, then

partially drying the coated fabric, and then before all the solvent has been evaporated subjecting the coated fabric to pressure to reduce the coating to the desired thickness.

5 2. The process of producing a coated fabric which comprises applying to a fabric a coating of a film-producing composition in the form of paste containing a solvent, then partially drying the coated fabric and 10 then before all the solvent has been evaporated subjecting the coated fabric to pressure between rolls to reduce the coating to the desired thickness.

3. The process of producing a coated fabric which comprises applying to a fabric a coating containing nitrocellulose and a solvent in the form of a paste, partially 15 evaporating the solvent of the paste, and

then before all the solvent is evaporated subjecting the coated fabric to pressure to reduce it to the desired thickness.

4. The process of producing a coated fabric which comprises applying to a fabric a coating containing nitrocellulose and a solvent in the form of a paste, partially 25 evaporating the solvent, and then before all the solvent has been evaporated passing the coated fabric between rolls to reduce it to the desired thickness.

In testimony that I claim the foregoing 30 I have hereunto set my hand.

CHARLES ELWOOD ARNOLD.

Witnesses:

H. W. MATHESON,  
HAMILTON BRADSHAW.